

C. A. PFANSTIEHL,  
METHOD OF PRODUCING HOLLOW OBJECTS OF COMPRESSED METALLIC POWDER,  
APPLICATION FILED NOV. 4, 1916.

1,286,089.

Patented Nov. 26, 1918.



Fig. 1



Fig. 2

Fig. 3

Witnesses:

Alvin C. Ahlberg.

Alfred S. Callaway

Inventor  
Carl A. Pfanstiehl  
By William Bradbury & Son  
Attorneys

# UNITED STATES PATENT OFFICE.

CARL A. PFANSTIEHL, OF HIGHLAND PARK, ILLINOIS, ASSIGNOR TO PFANSTIEHL COMPANY, INC., OF CHICAGO, ILLINOIS, A CORPORATION OF NEW YORK.

## METHOD OF PRODUCING HOLLOW OBJECTS OF COMPRESSED METALLIC POWDER.

1,286,089.

Specification of Letters Patent. Patented Nov. 26, 1918.

Application filed November 4, 1916. Serial No. 129,602.

To all whom it may concern:

Be it known that I, CARL A. PFANSTIEHL, a citizen of the United States, residing at Highland Park, in the county of Lake and State of Illinois, have invented a certain new and useful Improvement in Methods of Producing Hollow Objects of Compressed Metallic Powder, of which the following is a full, clear, concise, and exact description, reference being had to the accompanying drawings, forming a part of this specification.

My invention relates to a method of producing hollow objects of compressed metallic powder.

Tungsten and tantalum powders, magnesium oxid, tantalum oxid and thorium oxid and many other substances are useful in their compressed form as dishes in which to perform certain chemical operations, as heating elements in which to melt chemicals or metals. Some of these materials, especially tungsten and tungsten oxid, but many other materials to a less extent, resist flow during the compressing operation, that is, unless means are provided for compressing the material in substantially straight lines the material will become more highly compressed at one point than another, and will therefore be weak or porous at the points of less compression.

It has been found that tungsten powder and other powders, the particles of which are very hard, can be pressed into solid homogeneous objects by so distributing the tungsten or other powder under the movable part of the press that in the final position of the press all parts of the powder have received the same amount of compression. This is more readily accomplished where the article to be formed is rectangular in shape, since when in that shape only one of the dimensions of the loosely packed powder needs to be changed by the compression.

The pressure under which tungsten and some other powders are converted into solid homogeneous articles is about one hundred thirty to one hundred sixty tons per square inch. At such a pressure as this copper will flow and can even be squirted in a manner similar to that in which lead pipe and cable sheaths are made. By embedding a piece of copper in the powdered tungsten or other material to be compressed the cop-

per by its property of flowing exerts a lateral pressure upon the material being compressed and thus overcomes the characteristic of the tungsten or other powder which prevents it from flowing under pressure. 60

It has been found that although copper at the pressure of one hundred thirty tons per square inch and over will readily flow to equalize pressures throughout the powdered material being compressed, nevertheless the 65 tenacity of the copper is such as to prevent it from being forced into the pores of the powdered material under compression.

The shape of the copper invariably changes during the compressing operation 70 and the final shape to be secured must be determined by experimenting with different shaped copper inserts. Obviously, there are limitations to the shape which can be secured by means of the copper, but it has 75 been found that almost any form of smoothly outlined interior can be produced by this process.

The materials which I prefer to use in making chemical dishes and the like are not 80 readily attacked by the ordinary acids, whereas copper is readily attacked. The copper may therefore be removed by the use of nitric acid or if the powder be such as is attacked by nitric acid the copper may 85 be removed by some other acid which does not attack the compressed powder.

One form of my invention and one method of carrying it out are illustrated in the accompanying drawing, in which— 90

Figure 1 represents a collapsible die and its plunger filled with material for compression and also having the copper insert therein;

Fig. 2 is a section of the material after 95 compression; and

Fig. 3 is a perspective view of the material after the copper insert has been eaten out by the acid.

Similar characters of reference refer to 100 similar parts throughout the several views.

The die illustrated herein forms no part of my present invention, this die being the subject matter of my co-pending application, Serial No. 124,504, filed October 9, 105 1916, and entitled Means and method for compressing tungsten powder.

A die block 5 preferably of cast steel is provided with a plurality of removable members 6 having sloping faces which en- 110

gage correspondingly sloping faces of the die block. The members 6 are made of the hardest tool steel of which are also made the base member 7 and plunger 8. The base member 7 rests upon an insert 9 of steel which is somewhat harder than the cast steel block 5 but somewhat softer than the base member 7. Likewise the plunger 8 is carried in a supporting block 10 of steel which is somewhat softer than the plunger 8, but which is somewhat harder than the press member 11 in which the member 10 is supported. Suitable end members not shown are provided, these end members being likewise formed with sloping faces opposing the faces forming the walls of the die proper.

The rectangular chamber formed within the four walls and base of the die is filled 20 to the top with powder 13 to be compressed. The copper insert 14 is then forced into the powder until the upper and straight face of the copper insert is flush with the top of the die members 6. The plunger 8 is then 25 operated preferably by means of an oil pump and a pressure of substantially one hundred and fifty tons per square inch is exerted on the powder and copper. This pressure causes the copper to change its 30 form and to thus exert a lateral pressure substantially equal to the downward pressure exerted by the plunger.

After the compressing operation the pressure on the die members 6 is relieved by 35 backing off the screws 16 and 17, thus permitting the cross bar 18 to rise slightly, at the same time the pressure upon the plunger 8 is relieved, and the compressed material is allowed to expand. This expansion occurs 40 substantially equally in all directions, thus preventing the cracking of the compressed material.

The bar of material 19 with the copper 20 therein is placed in acid, the copper being 45 thus removed. The compressed material may then be washed and dried and used in its compressed form, or may thereafter be sintered by passing through it an electric current sufficient to bring the metal to its 50 welding temperature. Of course, if oxides are used they cannot be sintered in this manner, but if either metallic tungsten powder or metallic tantalum powder or in fact any metallic powder is used, the articles may 55 be sintered into solid metal. It is not always possible to perform this sintering operation by passing the electric current directly through the compressed material, because the material may by reason of its

shape have greater cross section at some 60 points than at others, by reason of which the resistance would be greater at some points than at others. The compressed object may, however, be supported upon a cradle of suitable material such as tungsten 65 rods, whereon the compressed article may be brought to a temperature sufficient to cause the particles to become sintered together.

Although but one form of compressed object is herein illustrated, it may readily be seen that other forms can be made by merely changing the shape of the die and the shape of the copper insert. It is possible also to use other metals than copper, though some 75 of the softer metals such as lead cannot readily be used, because the lead will be forced into the pores of the compressed material long before the necessary pressure has been reached to create a solid homogeneous article. When the soft metal is later eaten out of the pores the compressed material is left porous and therefore unfit for some purposes. If for any reason porous articles are desired, however, they may be constructed 80 by the use of lead or other very soft metals.

Having thus described my invention, what I claim as new and desire to secure by Letters Patent of the United States is:

1. The method of producing hollow articles of compressed metallic powders which consists in inserting a metal part having the property to flow under the pressure of compression, compressing the powder and metal 95 part and thereafter removing the metal part by the action of acids.

2. The method of producing hollow articles of compressed tungsten, tantalum, magnesium oxid, thorium oxid or the oxids 100 of tungsten and tantalum which consists in inserting a metal part within the unpacked powder to be compressed, compressing the powder about the metal part and thereafter removing the metal part.

3. The method of overcoming the characteristic of powdered tungsten and the like which prevents the powdered material from flowing under high pressure which consists in inserting within the material some other 110 metal which has the characteristic of flowing under pressure.

In witness whereof, I hereunto subscribe my name this 31 day of October, A. D. 1916.

CARL A. PFANSTIEHL.

Witnesses:

MARGARET GROBBEN,  
S. J. CRAIG.